

## UNITED STATES PATENT OFFICE

2,636,604

FLOTATION OF PYRITES FROM A PYRITE  
ORE PULPArvid Emil Anderson, Cornwall, Pa., assignor to  
Bethlehem Steel Company, a corporation of  
PennsylvaniaNo Drawing. Application June 17, 1949,  
Serial No. 99,883

2 Claims. (Cl. 209—166)

1

My invention relates in general to the concentration of mineral substances by froth flotation, and in particular to a flotation reagent for the recovery of iron pyrites ( $FeS_2$ ) and related sulphide ores.

In the froth flotation of iron pyrites, the reagents added to the aqueous ore pulp consist usually of copper sulphate ( $CuSO_4$ ), a collector or promoter, and a frother, which are separately fed to the pulp in a flotation machine in the order given. The copper sulphate is added in the form of a saturated water solution in amounts equivalent to 1.03 pounds per ton of dry feed, and simply cleanses the surface of the pyrite particles in aid of subsequent reactions. The collector brings together selectively the mineral particles to be recovered, while the frother creates the floating froth or foam which suspends the collected particles. Most reagents require the pulp to be heated for an effective separation. In some instances, activators or depressors are also added, ahead of the collector, but in nearly all cases the frother is added last.

I have discovered that the single addition of my improved pine oil-resinate-xanthate-water emulsion will simultaneously perform the functions of collector and frother, and will produce a more selective and powerful reaction with the sulphide minerals than previous reagents, with its effectiveness retained at lower temperatures.

The principal object of this invention, therefore, is an increased recovery of pyrites with decreased consumption and costs for reagents.

In accordance with my invention, a xanthate-resinate-pine oil-water emulsion of good stability is prepared, and this emulsion is added after the copper sulphate step to the pulp in the flotation operation, thus eliminating the additional two-step process of feeding the collector and frother separately.

To make 178.9 liters, or 47.08 gallons of my reagent, this being a convenient quantity for storage in a standard 50-gallon drum, 108 grams (3.81 oz.) of "Dresinate XXX" (trade name for sodium resinate) is dissolved in 10.8 liters (2.86 gals.) of G. N. S. No. 5 pine oil, to form a 1% (by weight) solution of "Dresinate" in pine oil. The resultant solution is added to 5.4 liters (1.43 gals.) of water and homogenized, under about 700 to 800 p. s. i. pressure, to form a "Dresinate"-pine oil-water emulsion resembling a thin marshmallow syrup. This first emulsion is then added to 108 liters (28.6 gals.) of a 25% (by weight) solution of sodium ethyl xanthate in water, together with an additional 5.4 liters (14.3 gals.) of wa-

2

ter, and the mixture is again fed through the homogenizer, with pressure set as before.

In other words, the proportions of the liquid constituents of the emulsion are substantially as follows: pine oil, 100 parts; sodium ethyl xanthate solution, 500 parts; and water, 300 parts.

The pine oil functions chiefly as a frothing agent, but as a practical matter it is almost impossible to form a stable pine oil-water emulsion without the help of an emulsifying agent. The addition of the small amount of "Dresinate XXX," however, produces a very stable emulsion and also improves the recoveries of pyrite. This emulsion, as mentioned above, is then further emulsified with the xanthate to form a xanthate-pine oil emulsion.

The major collecting effect is produced by the xanthate, which is the reaction product of an alkali metal hydroxide, carbon disulphide, and an alcohol. As stated, I prefer to use a 25% solution (in water) of sodium ethyl xanthate, which is the reaction product of sodium hydroxide, carbon disulphide, and ethyl alcohol, as the xanthate component, but sodium iso-propyl xanthate solutions, while somewhat less effective for the recovery of pyrite, may also be used with success. The reaction of the xanthate with the collected pyrite is to form an insoluble xanthate which is "air avid" and hence is strongly attracted to the bubbles of the froth.

This emulsion does not show the effects of decomposition or loss of strength over ordinary periods of time, as is normally the case with xanthates, and mixes very evenly and quickly with the feed. Actual plant tests indicate that an increase in pyrite recovery of about 3%, with about 10% less reagent, is readily attained with its use in conventional types of flotation machines.

Although I have thus described my invention in considerable detail, I do not wish to be limited to the exact and specific details shown and described, but may use such substitutions or equivalents thereof as are embraced within the scope of the invention or pointed out in the appended claims.

I claim:

1. A method of recovering pyrites from a pyrite ore pulp which comprises adding to the pulp an emulsion of a xanthate, pine oil, and sodium resinate, and subjecting the pulp to a flotation operation.

2. A method of recovering pyrites from pyrite ore pulps which comprises adding to the pulps an emulsion of sodium ethyl xanthate, pine oil, and

sodium resinate, and subjecting the pulps to a froth flotation operation.

ARVID EMIL ANDERSON.

References Cited in the file of this patent

UNITED STATES PATENTS

| Number    | Name               | Date           |
|-----------|--------------------|----------------|
| 1,547,732 | Broadbridge et al. | July 28, 1925  |
| 1,554,216 | Keller             | Sept. 22, 1925 |
| 1,992,949 | Hodges             | Mar. 5, 1935   |
| 2,116,727 | Lenher et al.      | May 10, 1938   |

| Number    | Name  | Date          |
|-----------|-------|---------------|
| 2,259,420 | Hills | Oct. 14, 1941 |
| 2,286,374 | Ray   | June 16, 1942 |

OTHER REFERENCES

5 Weinig et al. "The Trend of Flotation," Quarterly of the Colorado School of Mines, vol. XXXII, No. 4, 1937, page 59.

10 Bureau of Mines Bulletin 449, Development and Use of Certain Flotation Reagents, 1944, pages 5, third paragraph; and pages 76-79.